

Sept. 1, 1925.

1,551,536

A. G. CAMPBELL

METHOD OF TREATING CRUDE SULPHIDE ORES CONTAINING LEAD FOR THE  
RECOVERY OF HYDRATED CARBONATE OF LEAD AND BY-PRODUCTS

Filed July 12, 1922



Inventor:  
Alexander George Campbell  
By - P. Swiger, Atty

## UNITED STATES PATENT OFFICE.

ALEXANDER GEORGE CAMPBELL, OF BROKEN HILL, NEW SOUTH WALES, AUSTRALIA.

## METHOD OF TREATING CRUDE SULPHIDE ORES CONTAINING LEAD FOR THE RECOVERY OF HYDRATED CARBONATE OF LEAD AND BY-PRODUCTS.

Application filed July 12, 1922. Serial No. 574,562.

*To all whom it may concern:*

Be it known that ALEXANDER GEORGE CAMPBELL, a subject of the King of Great Britain, residing at Broken Hill, in the State of New South Wales (formerly of "Kia-Ora" Bay Road, Sandringham, in the State of Victoria), Commonwealth of Australia, has invented certain new and useful improvements in improved method of treating crude sulphide ores containing lead for the recovery of hydrated carbonate of lead and by-products, of which the following is a specification.

The present invention provides for the recovery of white lead and silver from crude sulphide ores containing sulphides of silver lead and zinc, or concentrates middlings or by products obtained from the treatment of such ores.

It is the purpose of this invention to leave the zinc, at the end of the process, in its unaltered condition as a sulphide.

At the present time there are numerous inventions and processes which relate to the production of white lead by what are known as precipitation processes, that is to say, processes in which the lead is first dissolved in a solution such as acetic acid, or of an alkaline salt, or some other solvent, and from which it is precipitated as a hydrated carbonate by various methods. Also among these precipitation processes there are some which make use of well known electrochemical reactions whereby an anode of metallic or pig lead is dissolved by the action of an electric current passing through a suitable electrolyte, while a caustic alkali is produced at the same time at the cathode, to be used, either directly or indirectly, to precipitate the lead from its solution.

In all precipitation processes, whether the lead is dissolved by electrolysis or other means, there are serious disadvantages, the greatest being that the solution is produced by dissolving metallic lead, involving the costly processes of smelting and refining of lead ores before the manufacture of white lead is even commenced, while it has hitherto been found extremely difficult to produce a product showing an amorphous structure

under the microscope, which is a desirable feature.

It is the aim of this invention to produce a white lead of good quality by direct treatment of a sulphide ore, by hydro-metallurgical methods, eliminating the expensive and unnecessary processes at present involved in the production of metallic lead.

To effect this a series of three steps are involved which include:—

First. Subjecting the ore to a process whereby the lead and silver values become contained as chlorides in an alkali metal chloride solution.

Secondly. Treating the solution for the elimination of impurities.

Thirdly. Precipitating the lead in solution as a hydroxide, which is then converted to a hydrated carbonate of lead.

Although this series of related steps is hereinafter claimed in combination, certain factors arise as will be evident from the following description which involve specific claims for certain methods of performing all or individual steps in the entire treatment.

Also, in the following description, it will be shown how, by a particular application to this process of a well known electrochemical method of producing caustic soda and chlorine by the electrolysis of a brine solution, the supply both of chloridizing agent and caustic soda may be regenerated at one and the same time.

The accompanying drawing is a vertical longitudinal sectional view of apparatus which may be employed in carrying out my process.

One object of my invention is to provide an improved process by which to make commercially possible the treatment of zinc ores and concentrates for the recovery of silver and lead values, which it would otherwise be unprofitable to extract, and which because associated with zinc would have little or no value.

To effect the first of the above specified steps the material is first crushed and ground, and then subjected to a preferential chloridizing roast whereby the lead and

55

60

65

70

75

80

85

90

95

100

silver values are converted to chlorides while the zinc remains substantially unaltered as a sulphide.

There are already methods in existence whereby this object may be attained. Thus the material may be roasted, under suitable conditions of temperature and time, with chloridizing agents such as metallic chlorides or hydrochloric acid, without the presence of oxidizing agents, or with an alkali metal chloride such as common salt, in an oxidizing atmosphere.

In all these methods, when the temperature is maintained within certain limits, the lead and silver values may be chloridized without affecting the zinc but there is a disadvantage which lies in the expense of a chloridizing agent.

As will be later described, my special and novel method of precipitation, used in this particular modification of the process, involves at the same time the production of an equivalent amount of chlorine, and for this reason the preferential chloridizing roast is carried out in the presence of chlorine. The ore, after having been crushed and ground, is roasted in an atmosphere of chlorine, in a suitable furnace or heated containing vessel at such a temperature as to convert the lead and silver values to chlorides, but to leave the zinc sulphide unaltered. Now though successful chloridizing of the lead and silver may be done by this means, there is a loss of chlorine due to its leaving the furnaces as gaseous chlorides of sulphur, and to prevent this it is preferable to add moisture in the form of steam, and also air, to the furnace atmosphere so that the chlorides of sulphur having been broken up by steam, the sulphur may be oxidized to sulphur dioxide gas.

In the treatment with chlorine as described it is essential that the temperature of the reaction be maintained within certain limits. This temperature will vary with different classes of ore and should be ascertained by direct experiment on a sample beforehand, but generally it has been found that a temperature of between 400° C. and 500° is sufficient. Also the amount of steam added should be sufficient only to break up the chlorides of sulphur formed by the action of chlorine on the sulphides. On the other hand the air, to complete the oxidation of sulphur, may be added slightly in excess without causing the formation of sulphates of either lead, silver or zinc. This method of preferential chloridizing of an ore by roasting, with chlorine to which steam and air has been added differs essentially from methods using hydrochloric acid alone in that steam and chlorine are employed as reagents instead of hydrochloric acid, that any hydrochloric acid formed by the action of steam on chlorine or chlorides of sulphur

play only a secondary part in the reaction, the main reagent being chlorine itself, and an oxidizing atmosphere is present for the purpose of oxidizing the sulphur, while in using hydrochloric acid alone, no oxidizing agent is used at all, the gas liberated being sulphuretted hydrogen.

Suitable means should be provided in roasting to rabble or otherwise keep the material in intimate contact with the furnace gases.

The roasted ore is now washed with warm water, by which the bulk of the chlorides of iron, manganese and copper are removed while the lead and silver chlorides, being practically insoluble remain unaltered.

These chlorides of lead and silver are now suitably leached, whereby the bulk of the lead but only a small and variably amount of silver chloride, unless measures are taken to increase its extraction, as later described, is brought into solution.

This solution, however carefully the roasted ore may have been originally washed, will usually be found to contain small quantities of impurities such as chlorides of iron, manganese or copper which must be removed if a pure white lead is to be produced. At this stage the performance of the second of above steps has now to be considered. Since the lead is ultimately to be precipitated as a hydroxide, it is essential that no reagent should be used to precipitate impurities which will itself form a soluble salt which will later be precipitated with and contaminate the white lead. For this reason the precipitants used for removing the impurities must be either metallic lead, or salts of lead, or sodium salts or salts of some base which will produce a salt in the solution which may be precipitated itself by a sodium or lead salt, or by some acid. Thus the silver may be precipitated by the known method of agitating the solution with granulated or sponge lead, whereby the lead and copper are precipitated in the metallic state. The lead with the deposit of silver and copper may be removed from time to time and smelted to produce a silver lead bullion.

Iron may be removed by agitation with powdered lead carbonate, whereby it is thrown down as an insoluble red precipitate, or iron and copper may be both removed as insoluble sulphides by agitation with powdered lead sulphide and this lead sulphide may be produced in the solution itself by a measured amount of sulphuretted hydrogen or a soluble sulphide such as sodium sulphide.

Iron and manganese together may be precipitated by suitable oxidizing agents such as red lead or lead peroxide.

In each of these cases when lead or a lead salt is used as a purifying agent, more lead chloride is kept hot and brought into

solution to be ultimately recovered in the form of white lead so that the expense of the cost of precipitants is counterbalanced by an increase in saleable product.

5 Both iron and manganese may also be removed from the solution by selectively precipitating them, with only a slight loss of lead, by adding an amount of an alkaline hypochlorite slightly in excess of the theoretical quantity required. A convenient means of obtaining an alkaline hypochlorite for this purpose is to agitate bleaching powder in the solution, in which case a certain amount of calcium chloride is brought into 10 solution.

15 This may be precipitated, without affecting the lead, as an insoluble sulphate by the addition of an equivalent amount of sodium sulphate or lead sulphate or sulphuric acid to the solution.

20 In using any one of these methods of purification the precipitant must be agitated by suitable means in the solution, which must be also filtered carefully after the 25 action is complete.

25 In addition to the above methods of purification a pure solution of lead chloride in brine may be obtained by crystallizing some of the lead by cooling, filtering, and 30 returning the solution for further leaching. The crystallized lead chloride may then be washed in pure water and re-dissolved in a separate brine circuit for further treatment.

35 The third of the above steps has now to be carried out.

40 The purified and hot solution of lead chloride in brine, after filtration, is passed into a suitable agitator or mixer where it is mixed with a solution of caustic soda, which, reacting with the lead chloride, 45 throws down an insoluble white precipitate of lead hydroxide and produces at the same time an equivalent amount of sodium chloride which thus regenerates the solution.

50 This precipitate may then be converted to a hydrated carbonate of lead by passing into it, while agitated, a stream of carbonic acid gas, and this operation is best carried out in a closed containing vessel to avoid loss of gas, the gas being introduced in measured quantity to supply whatever proportion of carbonic acid gas as may be desired. Generally the amount of gas introduced is equal to the theoretical amount given by the formula  $2\text{PbCO}_3\text{Pb}(\text{OH})_2$ , as white lead having this formula has been found to be of the best quality, but no particular amount is specified in this invention.

55 The process of introducing carbon dioxide gas into the precipitate may be carried out under pressure, in which case the reaction is more active, and it may also be carried 60 out by first filtering the hydroxide from the

brine solution and then mixing it with water in the agitator.

In precipitating the hydroxide from the brine solution by an alkaline metal hydroxide it has been found that a crystalline compound of the hydroxide with water has been apt to form, and that this combined water, after treatment of the precipitate with carbonic acid gas, is difficult to drive off when 70 drying by heat.

75 This formation of crystalline compounds has been found to be minimized by carrying out the precipitation in a solution which is heated to a temperature which will vary slightly according to its strength, and is 80 best found by direct experiment, although satisfactory results have been obtained with a number of solutions of varying strengths at  $75^{\circ}\text{C}$ .

85 The precipitated hydrated carbonate of lead, after careful washing and filtration, is slowly dried and is then in a condition to be ground in oil as commercial white lead.

90 This precipitate, obtained under these conditions, has been found to be equal in purity of color, covering power and amorphous structure with white lead made by the stack process.

95 The hydroxide of lead, formed by precipitation by a caustic alkali, may if desired be converted to a sulphate by digesting or heating with sulphuric acid, and this sulphate may be used as a pigment. Lead sulphate however, has only one advantage in 100 being nonpoisonous, while the hydrated carbonate, although a poisonous compound, has a greater spreading and covering power and for this reason is preferred to be manufactured as described.

105 The spent brine solution, after the removal of the precipitate, is then returned partly to the leaching circuit, while part is diverted to an electrolytic plant, where it passes through electrolytic cells, in which, by the 110 well known method of electrolysis, caustic soda is produced at the cathode and chlorine gas at the anode.

115 The chlorine gas is conveyed by pipes to the roasting furnace, while the mixed solution of brine and caustic soda enters the circuit again as a precipitant. It will thus be seen that the process is completely regenerative, the only agents to be purchased being electrical power, sufficient water to make up the amount lost in the form of lead hydroxide, and salt to make up unavoidable losses in washing, etc. It must also be pointed out that as a solution of caustic soda and brine is only required here, the usual costly processes in manufacture of caustic soda, of producing a solid product free from moisture and salt is dispensed with.

120 Though the method which has now been 125 described has been found, for the reasons 130

already given, to be economically the most suitable for carrying out the three steps mentioned above, it is not intended that it shall be binding to exclusion of other methods of carrying out the individual steps.

Thus silver and lead may be obtained as chlorides in an alkali metal chloride solution by other means, such as by known wet methods, and the lead precipitated from 10 the purified solution by some alkaline hydroxide such as ammonium hydroxide which will precipitate the lead but not throw down the base of the chloride used as a solvent.

Of available hydroxides it has been found 15 that lime is so slightly soluble and has such a tendency to form oxychlorides of lead that it is impracticable, while potassium is usually too expensive.

Ammonium hydroxide may be used with 20 cold solutions, to prevent its breaking up by heat, and may be recovered from the leach solution, after filtration of the precipitate, by digesting while heated with lime, the fumes of ammonia, given off being collected 25 for further use, while the solution gains an equivalent increase in calcium chloride.

This method involves the use of large volumes of solution, as calcium chloride has a lower solvent power of lead chloride than 30 brine especially when cold while it is difficult also to avoid losses of ammonia.

It will thus be seen that, provided power may be obtained at a reasonable cost, the particular method detailed, that is the use 35 of a brine solution and caustic soda as a precipitant, has the greatest advantages.

It will also be obvious that there may be occasions, when dealing with certain ores, there will be no necessity for purifying the 40 leach solution, but the elimination of this step does not necessarily alter the principle of this invention.

In the leaching of the roasted ore it has been found that however well the silver values 45 may have been chloridized, that only a small amount may be brought into solution owing to the fact that being in contact with zinc sulphide it reverts itself to a sulphide. This difficulty in leaching silver in the presence of unaltered zinc sulphide has been known for a long time and various mechanical methods have been devised to overcome it, the principle being to remove the silver chloride, when once in solution, as soon as 50 possible from contact with the zinc sulphide by such methods as rapidly passing the solution through the beds of ore on filter beds, or by the use of suction filters or centrifugal extractors or the like.

These methods have all a fundamental disadvantage in that the silver is only removed after it has dissolved and is so in a state in which it can react with the zinc sulphide and a special method according to 55 this invention will now be described where-

by the silver and lead chlorides are largely removed from contact with the zinc sulphide before being dissolved at all.

This method consists in pouring a stream 70 of roasted ore on to the surface of a moving stream of leach solution so that the particles of zinc sulphide, sinking at a faster rate than the particles of chlorides, are rapidly and simply removed from contact 75 with the silver in solution. The attached sectional elevation will shew a simple and convenient means by which this can be effected, the description being as follows:—  
(1) is a small hopper into which the washed 80 ore is placed and by means of a spray of hot brine from the pipe (2) is washed in a thin stream on to and across the surface of the solution in the leaching trough (5).

The hot leaching solution is introduced 85 into this trough by means of the pipe (3) and by the perforated baffle (4) is distributed evenly. This stream of hot solution flows through the trough as shewn by the arrows, to the perforated baffle (6) and 90 then out of the trough by the pipe (7).

When the washed ore flows on to the surface of the leach solution the particles of zinc sulphide sink evenly through the solution and more quickly than the particles of chlorides. These becoming smaller and 95 smaller as they dissolve, sink more and more slowly so that by the time the zinc sulphide has fallen to the bottom the operation is complete and the chlorides leave the trough 100 dissolved in the solution.

The zinc sulphide residue is removed by the plug holes 8, while the depth of flow of solution may be controlled by covering the perforations in the baffles by means of 105 the slats fixed in grooves, one of which is shewn in the diagram at the exit.

By this means a higher extraction of silver may be obtained than by other mechanical methods, while the time and expense of the operation is largely reduced. As an alternative method of recovering the silver, the ore may be leached first for lead and the silver afterwards leached from the zinc residue by known solvents which will 110 dissolve silver sulphide, such as a solution of a double hyposulphite of sodium and copper, or by chlorine in a brine solution, or by a solution containing a metal forming higher and lower chlorides and saturated 115 with chlorine.

As an example of the use of chlorine for the preferential roasting of a silver-lead-zinc ore, a sample of silver lead zinc middlings assaying 25.8 oz. silver, 36.8% lead, 24.7% zinc was roasted in an atmosphere 120 of chlorine for a period of one and a half hours, at a temperature not exceeding 450° centigrade. The roasted material was then leached with known solvents when the residue 125 was found to assay 2.9% lead.

Another sample of the same material was then roasted under the same conditions but with the addition of steam and air to the furnace atmosphere. The residue, after 5 leaching, was found to contain 0.6% lead. In each case the zinc sulphide was found to be substantially unaltered.

I claim:-

1. A method for the production of white lead from crude ore or concentrates containing lead, by first chloridizing the silver and lead values and then leaching these values by a solution of an alkali metal chloride, secondly purifying this solution, and finally

precipitating the lead as a hydrated carbonate by the addition of an alkali metal hydroxide followed by agitation with a stream of carbonic acid gas.

2. Producing white lead from crude ore or concentrates, by a preferential roast with chlorine, leaching the lead and silver chlorides by a solution of brine, purifying this solution, and precipitating the lead as a hydrated carbonate by means of caustic soda and carbonic acid gas.

25

Dated this 16th day of May 1922.

ALEXANDER GEORGE CAMPBELL.